

## UNITED STATES PATENT OFFICE

1,941,475

## BLEACHED CONDENSATION PRODUCT OF CARBOHYDRATES AND CRUDE HYDROCARBONS

Alphons O. Jaeger, Mount Lebanon, and Heinrich W. Witzel, Ingram, Pa., assignors to The Selden Company, Pittsburgh, Pa., a corporation of Pennsylvania

No. Drawing: Application February 25, 1931  
Serial No. 518,291

4 Claims. (Cl. 260—2)

This invention relates to condensation products of carbohydrates, aromatic hydrocarbons and sulfuric acid which may or may not also contain organic acids such as phthalic anhydride, 5 aldehydes, or both.

In co-pending applications of Jaeger, Serial No. 512,500 filed January 30, 1931; Serial No. 512,752 filed January 31, 1931; and Serial No. 512,753 filed January 31, 1931, condensation products of crude 10 aromatic hydrocarbons or residues from the purification of aromatic hydrocarbons are condensed with carbohydrates and sulfuric acid or with carbohydrates treated with phthalic anhydride and sulfuric acid, the products being tanning agents.

15 While the tanning power of the products is excellent and the raw material is very cheap, many of the products are open to the objection that they are highly colored, this being particularly true of the products obtained from crude residues 20 from the purification of aromatic hydrocarbons, some of which are black or very dark brown and are, therefore, objectionable when used with light colored leathers.

Similarly, tanning agents obtained by the sulfonation of crude aromatic hydrocarbons or other residues which are described in the co-pending application of Jaeger and Witzel, Serial No. 518,- 25 292 filed February 25, 1931 are likewise very dark in color. The condensation products of cellulose, crude aromatic hydrocarbons and sulfuric acid when reacted with aldehydes as described and 30 claimed in the application of Jaeger and Witzel, Serial No. 520,456 filed March 5, 1931 likewise present problems in tanning due to their high 35 color.

Tanning agents obtained by the sulfonation of crude coal tar fractions such as anthracene oil, etc. may likewise be bleached by the process of the present invention. These tanning agents 40 obtained by sulfonating crude coal tar fractions are described in the co-pending application of A. O. Jaeger, Serial No. 519,267 filed February 28, 1931.

According to the present invention, we have 45 found that, surprising as it may seem, the condensation products may be bleached with oxidizing agents, for example hypochlorites, either in the preformed state or formed in situ by the use of chlorine, which decolorize the highly colored products, transforming them into relatively light colored material, varying from a yellow to a light brown, which can be used even in the tanning of light colored leathers and which show no noticeable diminution in tanning power provided 50 the treatment is carried out carefully and no

great excess of oxidizing agent is used. If too large an excess of oxidizing agent is used the tanning power is lessened, and if a sufficient excess is used it may be entirely destroyed. While the amount of oxidizing agent will naturally vary to 60 some extent with the nature of the condensation product and its impurities, we have found that in general with condensation products containing cellulose and residues from the purification of aromatic hydrocarbons such as crude anthracene should not be treated with more than 50% of their weight of the oxidizing agent and usually 10% gives better results.

In addition to the hypohalites, other oxidizing agents may be used such as chlorine in acid solution, chromic acid, potassium permanganate, etc., and, if desired, mixtures may be used. In case of chromic acid, the reduction product is itself a tanning material.

The constitution of the condensation products 75 involved in the present invention is not definitely known and the action of the oxidizing agent is likewise not definitely proven. Nevertheless, we are of the opinion that the oxidizing agent, if not used in excess, acts primarily on certain colored 80 impurities of the condensation product. The invention is, of course, in no sense limited to this theory, which is merely advanced as apparently the most probable explanation of the action of the oxidizing agent in the present invention. 85

The invention will be described in greater detail in connection with the following specific examples.

## Example 1

50 parts of the black granular mass obtained according to Example 1 of the Jaeger application Serial No. 512,500 filed January 30, 1931 and which is the condensation product of the residue from the purification of crude anthracene by means of furfural, cellulose and sulfuric acid are mixed with 500 parts by weight of water and vigorously stirred for one hour. 400 parts of a water solution containing 10.84 parts of NaOCl is vigorously stirred in. The stirring is continued for about two hours, the color of the liquor changing from dark brown or black to dark yellow or very light brown. On evaporation, a solid is obtained which is readily soluble 105 in water and shows good tanning power.

Instead of using sodium hypochlorite, chlorine may be passed in, the solution being kept sufficiently alkaline to assure good absorption of the chlorine. The amount of chlorine passed in 110

should, of course, correspond to about 10% sodium hypochlorite.

Instead of using hypohalites, potassium permanganate or chromic acid may be used.

5

*Example 2*

A condensation product of cellulose, the residue from the vaporization of crude naphthalene and sulfuric acid, prepared according to Example 1 of the application of A. O. Jaeger, Serial No. 512,752, in the form of its sodium salt is treated as described in the foregoing example. The brownish black solution is changed to a deep yellow or brownish yellow, and, after evaporation, the material shows good tanning power, the tanning power being substantially as great as that of the unbleached material.

15

*Example 3*

A condensation product of cellulose treated with phthalic anhydride, the residue from the solvent purification of anthracene and sulfuric acid, prepared as described in Example 1 of the application of A. O. Jaeger, Serial No. 512,753 filed January 31, 1931, in the form of its sodium salt is treated with a hypochlorite as described in Example 1. A very marked lightening in color is obtained without substantially affecting the tanning power of the material.

20

*Example 4*

The condensation product of cellulose, the residue from the solvent purification of crude anthracene, sulfuric acid and formaldehyde, as described in Example 1 of the Jaeger and Witzel application Serial No. 518,292 filed February 25, 1931, above referred to, in the form of its sodium

25

30

35

40

45

50

55

60

65

70

75

or calcium salt is treated with a hypochlorite as described in Example 1. The brownish black liquor is transformed into a light brown or brownish yellow, and retains its tanning powers.

What is claimed as new is:

1. A process of producing light colored tanning agents, which comprises condensing at least one carbohydrate, phthalic anhydride and at least one impure aromatic hydrocarbon with sulfuric acid and subjecting a dispersion of the soluble condensation product obtained to the action of a bleaching agent in amounts sufficient to substantially lighten the color, but insufficient to destroy the tanning properties thereof.

2. A process of producing light colored tanning agents, which comprises condensing at least one carbohydrate, phthalic anhydride and at least one substance belonging to the group consisting of residues from solvent purification of crude anthracene with phenanthrene and carbazole solvents, residues from solvent purification of crude anthracene with phenanthrene solvents, residues from the vaporization of impure anthracene, residues from the vaporization of crude naphthalene, with sulfuric acid and subjecting a dispersion of the condensation product obtained to the action of a bleaching agent in amounts sufficient to substantially lighten the color, but insufficient to destroy the tanning properties thereof.

3. A process according to claim 1, in which the bleaching agent is a hypohalite.

4. A process according to claim 2, in which the bleaching agent is a hypohalite.

5. A process according to claim 1, in which the bleaching agent is a hypohalite.

6. A process according to claim 2, in which the bleaching agent is a hypohalite.

7. A process according to claim 1, in which the bleaching agent is a hypohalite.

8. A process according to claim 2, in which the bleaching agent is a hypohalite.

9. A process according to claim 1, in which the bleaching agent is a hypohalite.

10. A process according to claim 2, in which the bleaching agent is a hypohalite.

11. A process according to claim 1, in which the bleaching agent is a hypohalite.

12. A process according to claim 2, in which the bleaching agent is a hypohalite.

13. A process according to claim 1, in which the bleaching agent is a hypohalite.

14. A process according to claim 2, in which the bleaching agent is a hypohalite.

15. A process according to claim 1, in which the bleaching agent is a hypohalite.

16. A process according to claim 2, in which the bleaching agent is a hypohalite.

17. A process according to claim 1, in which the bleaching agent is a hypohalite.

18. A process according to claim 2, in which the bleaching agent is a hypohalite.

19. A process according to claim 1, in which the bleaching agent is a hypohalite.

20. A process according to claim 2, in which the bleaching agent is a hypohalite.

80

85

90

95

100

105

110

115

120

125

130

135

140

145

150